# EUROPEAN PATENT SPECIFICATION

(11) **EP 1 252 374 B1**
(45) Date of publication and mention of the grant of the patent: **23.04.2008**
(21) Application number: 00980265.3
(22) Date of filing: 21.11.2000
(51) Int. Cl.: C25D 21/14, C25D 21/18

(54) **PROCESS FOR THE EXTENDED USE OF ELECTROLYTES**
VERFAHREN FÜR DEN ERWEITERTEN GEBRAUCH VON ELEKTROLYTEN
PROCEDE D'UTILISATION PROLONGEE D'ELECTROLYTES

(30) Priority: 25.11.1999 DE 19956666
(43) Date of publication of application: 30.10.2002
(73) Proprietor: Enthone Inc., West Haven, Connecticut 06516 (US)
(72) Inventor: TOLLS, Elmar, deceased (DE); LUDWIG, Ralf, Wilhelm, 41516 Grevenbroich (DE); SCHÖNGEN, Gerd, 52499 Baesweiler (DE)
(74) Representative: Stenger, Watzke & Ring
(86) International application number: PCT/US2000/030148
(87) International publication number: WO 2001/038610

(56) References cited:
- DE-A- 2 015 739
- FR-A- 2 384 037
- US-A- 3 922 208
- US-A- 4 102 755
- US-A- 4 102 756
- US-A- 5 312 539
- US-A- 5 573 652
- US-A- 5 690 804
- US-A- 5 840 170

## Description

The invention refers to a process for the extended use of electrolytes, especially for depositing of non-glare metal coatings on a metal surface.

It is understood that metal coatings also include metal alloy coatings, and metal surfaces also include metallized surfaces of non-metallic objects.

The electrolytes used for plating generally are based on the customary, known composition components for the particular metal being plated. For example, in the case of nickel deposits from Watts nickel type electrolytes, these would be nickel sulfate, nickel chloride and boric acid.

Electrolytes based on chloride, sulfate, sulfamate, fluoroborate or mixtures thereof may be used for the metals nickel, copper, zinc, tin as well as for noble metals. In addition, the electrolytes may contain selected organic or inorganic base brighteners, grain improvers, brighteners or complexing agents.

In order to achieve absence of glare, a finely dispersed system is generated in the electrolyte by the addition of inorganic or organic foreign materials, so that these additives during the precipitation are either built into the deposit and/or interrupt for a short time the precipitation of the cathode film locally.

In the case of the known processes, finely ground insoluble materials, such as graphite, barium sulfate, aluminum oxide, glass etc. are added to the electrolyte. These products are maintained in suspension by strong agitation of the electrolyte and built into the deposit during the precipitation.

In modem processes the fine dispersal phase is generated in the electrolytes themselves. One or more surfactants are added to the solution which form a homogeneous solution below their cloud point, but form a finely dispersed emulsion above their cloud point.

As is the case with all emulsions, the stability of the fine dispersal phase is limited. Over time, the droplets increase in size and negatively affect the uniformity of the precipitation.

In practice, the emulsion is stabilized in that an electrolyte is continuously cooled to below the cloud point temperature, whereby the surfactant again goes into complete solution in the electrolyte. Subsequently, the electrolyte is again brought to the working temperature. The heating / cooling circuit required causes substantial additional operating cost.

If one works with an elevated salt content, the addition of a few milligrams per liter of selected surfactants already are sufficient to achieve a non-glare precipitation. Even without the forming of a visibly, cloudy emulsion, high-quality glare suppression is achieved. The surfactant may subsequently be readjusted several times, so that a worsening of the appearance of the layers due to coagulation occurs only after a period of 12 - 14 hours. The electrolyte functions without a secondary circuit. The coagulate may be removed by filtration over activated charcoal.

In addition, a fine dispersal phase may be generated by the reaction of soluble anionic and cationic combined with difficult-to-dissolve, higher-molecule salts in electrolytes. However, also in this case, after a working cycle of 8 - 10 hours the foreign material must be removed completely from the electrolytes by filtration due to coagulation effects. For the next working cycle the dispersion phase must be rebuilt again each time by the addition of components.

The higher-molecular compounds may also be directly added to the electrolytes.

Materials such as proteins or polysaccharides are present in aqueous solutions in colloidal form, and they lead to non-glaring coatings with suitable electrolyte compositions. These compounds are reduced by hydrolysis and/or reaction at the electrodes, and the glare removing property is increasingly destroyed.

The invention deals with the technical problem to prepare a process for the extended use of electrolytes which ensures a high electrolyte quality with a low economic investment, without having to accept production interruptions for regeneration.

Especially, it is envisaged to conduct the process for the precipitation of non-glaring metal coatings in such a manner that work can proceed in three shifts, five days per week without encountering production interruptions due to coagulation or destruction of the fine dispersal phase, respectively, and without the additional operating cost of a heating / cooling circuit.

The solution proposed by the invention is that during the continued use of an electrolyte a part of the flow is deviated, filtered and, if necessary, reconstituted by the addition of active substances and subsequently reintegrated in the operating cycle.

It is therefore suggested, in a partial flow of the electrolyte, to continually remove by filtration, wholly or in part, the coagulated particles and the not yet coagulated particles, as well as high-molecular compounds and their decay products, and that the appropriate quantity of additives is added to the filtrate prior to its reintegration.

Extended filtration means that filtration takes place primarily during the operating cycle.

A thorough cleaning of the electrolyte can be performed on weekends.

The invention describes a process for the extended use of electrolytes for the precipitation of non-glare metal coatings which, in addition to the metal salt, may also contain conducting salts, base brighteners, grain improvers and complexing agents in which a finely dispersed colloidal phase is generated in order to achieve non-glare properties. This is characterized by a partial flow of the electrolyte in which coagulated particles and not yet coagulated particles are removed wholly or in part by means of filtration and that an appropriate quantity of the active substances is subsequently added prior to reintegration.

A portion of the electrolyte can be directed into an overflow compartment for filtration. The overflow compartment should be able to contain between 5 and 25% of the actual bath volume.

Any type of filtration capable of removing very finely dispersed, finely dispersed and more grossly dispersed particles, wholly or in part, from the electrolyte may be employed. The different porosity of the filter materials and the use of filtration aids and/or activated charcoal may serve to differentiate between the various particle sizes.

Plate filters of defined porosity commonly employed in electroplating can be used, precoated with filtration aids and/or activated charcoal, as well as the common precoated multiple tube filters with defined porosity. Without precoating, wound tube filters may be used.

Also, classical methods of fractionating colloidal systems, such as dialysis, ultra and membrane filtration may be employed.

5 - 40% of the bath volume should be filtered per hour.

## Claims

1. A process for extending the use of non-glare metal plating to form a non-glare metal deposit which employs an electrolyte bath comprising a non-glare material tending to coagulate under the non-glare metal plating operating conditions, the process comprising:
a) deviating an electrolyte flow from the electrolyte bath;
b) filtering the electrolyte flow to remove particles of non-glare material which have coagulated under the non-glare metal plating operating conditions wherein the non-glare material constitutes additives which are intended either to be built into the metal deposit and/or to interrupt for a short time plating of the deposit locally; and
c) returning the filtered electrolyte flow to the electrolyte bath.

2. The process of Claim 1 wherein the non-glare material comprises a surfactant and wherein the non-glare metal plating operating conditions include operating at an electrolyte bath temperature above a cloud point temperature of the surfactant.

3. The process of Claim 1 wherein the electrolyte flow has a flow rate such that a volume of electrolyte between 5% and 40% of the volume of the electrolyte bath is filtered per hour.

4. The process of Claim 1 wherein the filtering step comprises a filtration process selected from the group consisting of precoated plate filtration, precoated multiple tube filtration, wound tube filtration, dialysis, ultra filtration, and membrane filtration.

5. The process of Claim 1 further comprising filtering the electrolyte flow to remove materials selected from the group consisting of uncoagulated glare-suppressing material, high molecular compounds, and decay products of high molecular compounds.

6. The process of Claim 1 further comprising the step of replenishing the electrolyte bath by adding an active substance to the electrolyte flow in an amount which is substantially equal to an amount of the active substance removed by consumption in the non-glare metal plating operation and by filtration from the electrolyte flow.

7. The process of Claim 6 wherein the active substance is selected from the group consisting of surfactants, metal salts, conducting salts, base brighteners, grain improvers, and complexing agents.

8. The process of Claim 6 wherein the active substance is added to the electrolyte flow after the filtering step and prior to returning the electrolyte flow the electrolyte bath.

9. The process of Claim 1 wherein the non-glare metal plating operation continually operates for a period of greater than 14 hours.

10. The process of Claim 1 wherein the non-glare metal plating operation continually operates for a period of greater than 5 days.

## Patentansprüche

1. Verfahren zur Verlängerung des Einsatzes einer galvanischen Abscheidung zur Bildung eines blendfreien metallischen Überzugs, wobei ein Elektrolytbad verwendet wird, das ein blendfreies Material enthält, welches unter den Einsatzbedingungen der blendfreien Galvanisierung dazu neigt, zu koagulieren, wobei das Verfahren umfasst:
a) Ableiten eines Elektrolytflusses von dem Elektrolytbad;
b) Filtern des Elektrolytflusses, um Partikel blendfreien Materials zu entfernen, die unter den Einsatzbedingungen der blendfreien Galvanisierung geronnen sind, wobei das blendfreie Material Additive bildet, die dafür vorgesehen sind, entweder in den metallischen Überzug eingebaut zu werden und/oder den galvanischen Niederschlag lokal für kurze Zeit zu unterbrechen; und
c) Rückführen des gefilterten Elektrolytflusses in das Elektrolytbad.

2. Verfahren nach Anspruch 1, wobei das blendfreie Material ein Tensid umfasst und wobei die Einsatzbedingungen der blendfreien Galvanisierung den Einsatz bei einer Temperatur des Elektrolytbads über einer Trübungspunkt-Temperatur des Tensids umfassen.

3. Verfahren nach Anspruch 1, wobei der Elektrolytfluss eine Durchflussrate derart aufweist, dass ein Elektrolytvolumen zwischen 5% und 40% des Volumens des Elektrolytbads pro Stunde gefiltert wird.

4. Verfahren nach Anspruch 1, wobei der Schritt des Filterns einen Filtrationsvorgang umfasst, der aus der Gruppe ausgewählt wird, die aus der Anschwemm-Plattenfiltration, Anschwemmfiltration mit Mehrfachfilterröhren, Anschwemmfiltration mit rohrförmigen Wickelelementen, Dialyse, Ultrafiltration und Membranfiltration besteht.

5. Verfahren nach Anspruch 1, ferner umfassend das Filtern des Elektrolytflusses, um Stoffe zu entfernen, die aus der Gruppe ausgewählt werden, die aus nichtkoagulierten blendunterdrückenden Stoffen, hochmolekularen Verbindungen und Zerfallsprodukten von hochmolekularen Verbindungen besteht.

6. Verfahren nach Anspruch 1, ferner umfassend den Schritt des Nachfüllens des Elektrolytbads durch die Zugabe einer aktiven Substanz zu dem Elektrolytfluss in einer Menge, die im wesentlichen gleich einer Menge der aktiven Substanz ist, die durch den Verbrauch bei dem Vorgang der blendfreien Galvanisierung und durch Filtration aus dem Elektrolytfluss entfernt wurde.

7. Verfahren nach Anspruch 6, wobei die aktive Substanz ausgewählt wird aus der Gruppe, die aus Tensiden, Metallsalzen, Leitsalzen, Basis-Glanzbildnern, Kornverbesserungsmitteln und Komplexbildnern besteht.

8. Verfahren nach Anspruch 6, wobei die aktive Substanz dem Elektrolytfluss nach dem Schritt des Filterns und vor der Rückführung des Elektrolytflusses in das Elektrolytbad zugegeben wird.

9. Verfahren nach Anspruch 1, wobei der Prozess der blendfreien Galvanisierung über einen Zeitraum von mehr als 14 Stunden beständig abläuft.

10. Verfahren nach Anspruch 1, wobei der Prozess der blendfreien Galvanisierung über einen Zeitraum von mehr als 5 Tagen beständig abläuft.

## Revendications

1. Procédé pour prolonger l'utilisation d'une opération de placage métallique anti-éblouissement pour former un dépôt métallique anti-éblouissement qui utilise un bain d'électrolyte contenant un matériau anti-éblouissement ayant tendance à coaguler dans les conditions de fonctionnement de l'opération de placage métallique anti-éblouissement, lequel procédé comprend :
a) la dérivation d'un flux d'électrolyte à partir du bain d'électrolyte;
b) la filtration du flux d'électrolyte pour éliminer les particules de matériau anti-éblouissement qui ont coagulé dans les conditions de fonctionnement du placage métallique anti-éblouissement, le matériau anti-éblouissement constituant des additifs destinés soit à être intégrés dans le dépôt de métal, soit à interrompre pendant une courte durée localement le placage du dépôt ; et
c) le renvoi du flux d'électrolyte filtré au bain d'électrolyte.

2. Procédé selon la revendication 1, dans lequel le matériau anti-éblouissement comprend un agent tensioactif et dans lequel les conditions de fonctionnement du placage métallique anti-éblouissement comprennent le fonctionnement à une température du bain d'électrolyte supérieure à une température de point de trouble du tensioactif.

3. Procédé selon la revendication 1, dans lequel le flux d'électrolyte a un débit tel qu'un volume d'électrolyte de 5 % à 40 % du volume du bain d'électrolyte soit filtré par heure.

4. Procédé selon la revendication 1, dans lequel l'étape de filtration comprend un procédé de filtration sélectionné parmi la filtration sur plaque pré-enduite, la filtration sur tubes multiples pré-enduits, la filtration sur tube en serpentin, la dialyse, l'ultrafiltration et la filtration sur membrane.

5. Procédé selon la revendication 1, comprenant en outre la filtration du flux d'électrolyte pour éliminer les matériaux sélectionnés parmi le matériau anti-éblouissement non coagulé, des composés de fort poids moléculaire et des produits de décomposition de composés de fort poids moléculaire.

6. Procédé selon la revendication 1, comprenant en outre l'étape de reconstitution du bain d'électrolyte par l'ajout d'une substance active au flux d'électrolyte dans une quantité substantiellement égale à une quantité de substance active soustraite par la consommation dans l'opération de placage métallique anti-éblouissement et par la filtration à partir du flux d'électrolyte.

7. Procédé selon la revendication 6, dans lequel la substance active est sélectionnée parmi les agents tensioactifs, les sels de métaux, les sels conducteurs, les brillanteurs de base, les agents améliorant le grain et les agents complexants.

8. Procédé selon la revendication 6, dans lequel la substance active est ajoutée au flux d'électrolyte après l'étape de filtration et avant le renvoi du flux d'électrolyte au bain d'électrolyte.

9. Procédé selon la revendication 1, dans lequel le placage métallique anti-éblouissement fonctionne en continu pendant plus de 14 heures.

10. Procédé selon la revendication 1, dans lequel le placage métallique anti-éblouissement fonctionne en continu pendant plus de 5 jours.
